

Nov. 4, 1924.

B. O. HENNING

1,513,989

METHOD OF DEOXIDIZING AND CLEANING METALS AND ALLOYS

Filed May 31, 1918

Fig. 1



Fig. 2



Inventor

Bertel O. Henning.

Charles J. Sherry,  
Atty

## UNITED STATES PATENT OFFICE.

BERTEL O. HENNING, OF CHICAGO, ILLINOIS.

## METHOD OF DEOXIDIZING AND CLEANING METALS AND ALLOYS.

Application filed May 31, 1918. Serial No. 237,386.

*To all whom it may concern:*

Be it known that I, BERTEL O. HENNING, a citizen of the United States, and a resident of Chicago, Cook County, and State of Illinois, have invented certain new and useful Improvements in the Method of De-oxidizing and Cleaning Metals and Alloys, of which the following is declared to be a full, clear, and exact description.

10 This invention relates to the method of deoxidizing and cleaning metals and alloys, and has for its primary object to greatly improve upon known methods for deoxidizing and cleaning metals and alloys, whereby maximum results may be obtained.

15 The casting of metals and alloys has brought out intensified study and application of various forms and practices with rather imperfect results.

20 Greater densities, homogeneity, closer grain, uniformity, tenacity, strength and conductivity have been sought, and attempts made to obtain the maximum of each element, by itself, or in combination as an alloy.

25 Oxides, gases and foreign matter in suspension in metal, and incomplete mixing of the molten metal are conceded as the causes of failure to obtain the maximum results.

30 Steam, if introduced into molten metal or alloy, causes violent agitation thereof, and serves as channels to carry the suspended matter to the top of the mass, the gases of which escape in the atmosphere and unreduced oxides and foreign matter remain floating on top.

35 One of the objects of this invention is to provide a method or process whereby metals and alloys can be purified and chemically mixed in their molten state, and as a consequence, in their solid state (when treated in accordance with the method of forming the subject matter of this application) become dense, homogeneous, uniform, tough, close grained and conductive to a greatly improved degree, and in a commercial and practical manner.

40 The invention consists in the hereinafter described method for deoxidizing and cleaning metals and alloys, which is more definitely defined in the claims.

45 An apparatus, whereby the method may be performed is illustrated in a drawing accompanying this specification, in which:—

Fig. 1 is a central, vertical section through

a melting kettle and showing in side elevation an apparatus for introducing the de-oxidizing and cleaning elements into molten metal, and Fig. 2 is a detail vertical section through a pump which forms part of the apparatus.

50 The method forming the subject matter of this invention, is to first dissolve boric acid (or any other deoxidizing agent which is soluble in water or other liquid) in a liquid, such as water (preferably distilled) either to saturation or a less degree depending upon the metal element or alloy to be treated. Secondly, the temperature of this solution is raised to a degree where the boric acid volatilizes and the water is generated into steam and this result can be obtained by passing the solution through a steam generator, such as for instance as a coil of pipe immersed in the molten metal contained in a melting kettle, pot, crucible, smelter or the like. The solution, coming in contact with the heat of the molten metal or alloy, causes the boric acid to volatilize and the water to vaporize, and both being released into the body of the molten metal or alloy, liberates the suspended metal oxides and other impurities from the metal or alloys. As the volatilized and vaporized solution rises to the top, it agitates the mass, mixes and purifies and drives to the top, the impurities held in suspension.

55 In the apparatus illustrated for carrying on this method, the reference character 5 designates a melting kettle of ordinary and well known form, supported on a wall 6. Heat may be supplied from a burner 7, below the kettle. A container for the solution is seen at 9, supported from the wall 6 by a bracket 8. In the container 9, is a plunger 14, which is operated by a stem 18, preferably screw threaded and mounted in a support 24, secured to the container. A screw threaded stem is preferable because it provides a slow movement for the plunger. A tube 11, of very small diameter is connected to the discharge end of the container and leads to the kettle 5 when it terminates in a steam generator or coil 31, which is immersed in the metal contained in the kettle. In the end of the coil is a discharge aperture. Said tube is practically a capillary tube to permit the flow of a very small body of the solution through it, and the steam generator is provided with a large heat radiating surface to insure the generation of vapors there-

in. The solution is introduced to the molten metal by turning up the screw threaded stem 18, of the plunger, which forces the solution out into the tube to the steam generator. I  
5 do not desire to limit myself to this form of apparatus, because other forms may be used, but it serves for the purpose of illustration.

The exact proportions of the elements employed for carrying on this process are not  
10 material, but the solution may be a saturate or only a partial saturate depending on the metal or alloy treated. Obviously other deoxidizing agents, which are soluble in water or other liquids, whereby the solution may  
15 be introduced into the molten mass in a volatilized and vaporized condition, may be substituted for boric acid, and I desire therefore, not to limit myself to the use of boric acid, but claim the use in this method of  
20 equivalent deoxidizing agents.

I claim as new and desire to secure by Letters Patent:

1. The method of deoxidizing and cleaning metals and alloys, which consists in introducing a mixture of steam and volatilized boric acid into the molten metal or alloy. 25

2. The method of cleaning metals and alloys, which consists in introducing a mixture of steam and a volatilizable metal cleaning agent, which is soluble in liquid, into the molten metal or alloy. 30

3. The method of cleaning metals and alloys, which consists in introducing a mixture of steam and any soluble metal cleaning 35 agent, into the metal or alloy while in a molten state.

4. The method of cleaning metals and alloys which consists in introducing a mixture of steam and a dissolved volatilizable metal 40 cleaning agent, into the molten metal or alloy.

BERTEL O. HENNING.